

# UNITED STATES PATENT OFFICE.

JOSEPH KINTZ, OF WEST MERIDEN, CONNECTICUT, ASSIGNOR TO HIMSELF  
AND PATRICK J. CLARK, OF SAME PLACE.

## PROCESS FOR COATING METAL CASTINGS.

SPECIFICATION forming part of Letters Patent No. 224,925, dated February 24, 1880.

Application filed July 1, 1879.

*To all whom it may concern:*

Be it known that I, JOSEPH KINTZ, of West Meriden, in the county of New Haven and State of Connecticut, have invented a new and

5 Improved Process for Coating Metal Castings, of which the following is a specification.

My invention consists in an improved process for giving an ornamental surface or finish to iron castings, which process is as follows:

- 10 The casting is first rolled or tumbled in the usual manner, and polished on the portions of the surface that are to have a polish on the finished article, and then the casting is coated with copper or other metal by electroplating.
- 15 It is next subjected to acid-bath, for cleaning, and then buffed to render the surface smooth and bright. It is then boiled in a tin or other metallic solution. The solution will deposit evenly over the entire surface, and the polished
- 20 portions will be left brilliant, thereby forming a fine contrast with the unpolished surface and giving a fine finish and effect.

The polishing previous to the electroplating, and the buffing subsequent thereto, are

essential steps in the process, and by the boiling 25 in a metallic solution the desired color and a bright clean finish are obtained without further labor.

The process is especially applicable to small castings in iron; but I do not limit myself in 30 that respect, nor to any special metallic solution for giving the finishing color.

I am aware that buffing, polishing, and plating are not new; but

What I do claim as new, and of my invention, is—

In the process of polishing and plating metals, a sub-process that consists in dipping the polished and plated metal in an acid mixture to brighten the ornamental part, then 40 buffing the plain surface, and finally boiling it in a metallic solution to produce a lively color.

JOSEPH KINTZ.

Witnesses:

WILBUR F. DAVIS,  
CHARLES W. MANN.